

# UNITED STATES PATENT OFFICE.

MAX FREMERY, OF OBERBRUCK, AND EMILE BRONNERT, OF MÜLHAUSEN-NIEDERMORSCHWEILER, GERMANY, AND JOHANN URBAN, OF ST. POLTEN, AUSTRIA-HUNGARY.

## PROCESS FOR THE MANUFACTURE OF THREADS, FILMS, OR OTHER FORMS OF CELLULOSE.

No. 856,857.

Specification of Letters Patent.

Patented June 11, 1907.

Application filed May 8, 1905. Serial No. 259,477. (Specimens.)

*To all whom it may concern:*

Be it known that we, MAX FREMERY and EMILE BRONNERT, both subjects of the German Emperor, and JOHANN URBAN, a subject of the Emperor of Austria, residing, respectively, at Oberbruck, Province of the Rhine, in the German Empire, Mülhausen-Niedermorschweiler, Alsace, in the German Empire, and St. Polten, in the Austrian Empire, have invented certain new and useful Improvements in Processes for the Manufacture of Threads, Films, or other Forms of Cellulose, of which the following is a specification.

15 Artificial silk has been made by injecting solutions of cellulose, in suitable solvents therefor, into agents which precipitate or coagulate the cellulose, for instance acetic acid or sulfuric acid of 30-65 per cent strength. 20 Silk-like cellulose threads have also been made by injecting a cupriferous ammoniacal solution of cellulose into a preferably weak solution of caustic soda and then removing the copper with which the cellulose thread is 25 mixed, by washing with an acid. When it is attempted, however, to make thick threads such as are suitable as a substitute for horse-hair, by either of these methods, the product is always dull, brittle and without the flexibility of natural horse-hair.

The present invention consists in the application of the surprising discovery that when an ammoniacal cupriferous solution of cellulose prepared at a low temperature, that is to 35 say, at a temperature below 10° C., as described in Patent No. 617,009, is subjected through a suitable opening, such as a slit or a comparatively wide cylindrical orifice into a strong caustic alkali solution, that is to say, 40 a solution having a specific gravity between 1.280 and 1.320; the film produced in one case and the thick thread in the other are brilliant, strong and elastic, and are moreover, water-proof even when they have been 45 washed with acid to remove the copper they

contain. Thus the thick threads made in one operation, that is to say, without spinning several fine threads together as has been customary heretofore, are excellently suited as substitutes for horse-hair. 50

The following examples illustrate the invention.

Example I. 240 kilos of cellulose, previously treated successively with a cold concentrated solution of caustic soda and an 55 oxidizing bleaching agent as described in U. S. Patent Specification No. 646351 are dissolved in, say 3000 liters of a cupriferous ammoniacal solution at a low temperature in the usual manner and the solution is injected through 60 capillary tubes into a strong solution of caustic soda, preferably a cold solution containing not less than 20 per cent. The threads of coagulated cupriferous cellulose thus produced are wound up in the usual manner, washed 65 with water until free from adhering caustic soda, and dried under tension.

Example II. A solution made by dissolving cellulose in a concentrated solution of cupric carbonate in a solution of ammonia of 70 about 16-18 per cent strength in the cold as described in U. S. Patent Specification No. 672350 is injected through a slit-shaped opening into caustic soda solution preferably a cold solution containing not less than 20 per 75 cent. The film of coagulated cupriferous cellulose thus produced is washed, laid between paper sheets and together with these rolled firmly on a cylinder or pressed, so that it may not suffer change of form, and dried. 80 Under certain circumstances it may be desirable that the copper contained in these products should be hidden. Thus the color of the product may be varied by treatment of the latter with sulfureted hydrogen, sulfuric acid, a solution of chromic acid or the like, in the known manner. This however is not essential to the invention. 85

Having thus described the nature of our said invention and in what manner the same 90

is to be carried into practical effect, we claim:—

1. A process for the manufacture of thick threads or films of cupriferous cellulose consisting in injecting into a strong solution of caustic alkali of about 1.3 specific gravity a solution of cellulose in cupriferous ammoniacal solution prepared at a temperature below 10° C., washing the coagulated cellulose thus obtained and drying it under tension.
2. A process for the manufacture of thick threads or films of cupriferous cellulose consisting in injecting into a strong solution of caustic soda of about 1.3 specific gravity a solution of cellulose in a cupriferous ammoniacal solution prepared at a temperature below 10° C., washing the coagulated cellulose thus obtained and drying it under tension.

In testimony whereof we have signed our names to this specification in the presence of 20 two subscribing witnesses.

MAX FREMERY.

EMILE BRONNERT.

JOHANN URBAN.

Witnesses to the signature of Max Fremery:

HENRY QUADFLIEG,  
GERARD SELLERS.

Witnesses to the signature of Emile Bronnert:

ALBERT GRAETER,  
GEO. GIFFORD.

Witnesses to the signature of Johann Urban:

ALVESTO S. HOGUE,  
AUGUST FUGGER.